



US008659217B2

(12) **United States Patent**  
**Kim et al.**

(10) **Patent No.:** **US 8,659,217 B2**  
(45) **Date of Patent:** **Feb. 25, 2014**

(54) **ARTICLE COMPRISING METAL OXIDE NANOSTRUCTURES**

(75) Inventors: **Dong-Wook Kim**, San Diego, CA (US);  
**Sungho Jin**, San Diego, CA (US);  
**In-Kyung Yoo**, Yongin-shi (KR)

(73) Assignees: **The Regents of the University of California**, Oakland, CA (US);  
**Samsung Electronics Co., Ltd.**, Gyeonggi-do (KR)

(\*) Notice: Subject to any disclaimer, the term of this patent is extended or adjusted under 35 U.S.C. 154(b) by 367 days.

(21) Appl. No.: **11/892,737**

(22) Filed: **Aug. 27, 2007**

(65) **Prior Publication Data**

US 2008/0054790 A1 Mar. 6, 2008

**Related U.S. Application Data**

(62) Division of application No. 11/059,784, filed on Feb. 17, 2005, now Pat. No. 7,276,389.  
(60) Provisional application No. 60/547,689, filed on Feb. 25, 2004.

(51) **Int. Cl.**  
**H01J 1/62** (2006.01)

(52) **U.S. Cl.**  
USPC ..... **313/491**; 428/615

(58) **Field of Classification Search**  
USPC ..... 313/495-497, 306, 309-310, 293-304;  
438/22, 34; 445/24; 428/615

See application file for complete search history.

(56) **References Cited**

U.S. PATENT DOCUMENTS

|                |         |                           |
|----------------|---------|---------------------------|
| 5,079,112 A    | 1/1992  | Berger et al.             |
| 5,532,496 A    | 7/1996  | Gaston                    |
| 5,654,497 A    | 8/1997  | Hoffheins et al.          |
| 5,735,721 A *  | 4/1998  | Choi ..... 445/24         |
| 5,982,095 A    | 11/1999 | Jin et al.                |
| 6,036,774 A    | 3/2000  | Lieber et al.             |
| 6,091,190 A    | 7/2000  | Chalamala et al.          |
| 6,129,901 A    | 10/2000 | Moskovits et al.          |
| 6,231,744 B1   | 5/2001  | Ying et al.               |
| 6,283,812 B1   | 9/2001  | Jin et al.                |
| 6,297,592 B1   | 10/2001 | Goren et al.              |
| 6,504,292 B1 * | 1/2003  | Choi et al. ..... 313/310 |

(Continued)

FOREIGN PATENT DOCUMENTS

|    |                 |        |
|----|-----------------|--------|
| JP | 2003-141986     | 5/2003 |
| KR | 10-2002-0049630 | 6/2002 |

(Continued)

OTHER PUBLICATIONS

Flahaut et al., "Carbon nanotube-metal-oxide nanocomposites: Microstructure, electrical conductivity and mechanical properties", Acta Materialia, pp. 3803-3812, 2000.\*

(Continued)

*Primary Examiner* — Nimeshkumar Patel

*Assistant Examiner* — Jacob R Stern

(74) *Attorney, Agent, or Firm* — Harness, Dickey & Pierce, P.L.C.

(57) **ABSTRACT**

This invention includes field emitters, in particular, electron field emitters with metal oxide nanoscale, aligned and sharped-tip emitter structures, the metal oxide emitter structures being a plurality of carbon nanostructures supported by and projecting from a substrate and including a metal oxide coating overlying the surfaces of the plurality of carbon nanostructures.

**14 Claims, 10 Drawing Sheets**



(56)

## References Cited

## U.S. PATENT DOCUMENTS

- 6,649,403 B1 11/2003 McDevitt et al.  
 2002/0076846 A1\* 6/2002 Ihm ..... 438/34  
 2003/0098518 A1\* 5/2003 Averdung et al. ..... 264/10  
 2003/0143581 A1\* 7/2003 Franzen et al. ..... 435/6  
 2003/0180472 A1\* 9/2003 Zhou et al. ..... 427/430.1  
 2003/0217586 A1\* 11/2003 Gouma ..... 73/31.06  
 2004/0071951 A1\* 4/2004 Jin ..... 428/323  
 2004/0157449 A1\* 8/2004 Hidaka et al. ..... 438/689  
 2004/0175844 A1\* 9/2004 Yang et al. ..... 438/2  
 2004/0191698 A1\* 9/2004 Yagi et al. ..... 430/320  
 2004/0262636 A1\* 12/2004 Yang et al. ..... 257/200  
 2005/0104056 A1 5/2005 Nihei  
 2006/0282225 A1\* 12/2006 Sunshine et al. ..... 702/32

## FOREIGN PATENT DOCUMENTS

- KR 10-2003-0060611 7/2003  
 KR 10-2003-0084279 A 11/2003  
 KR 10-2003-0097125 A 12/2003  
 KR 10-2004-0079226 A 9/2004

## OTHER PUBLICATIONS

- Zhao, L.; Gao, L. Carbon 2004 42 3269 3272.\*  
 Korean Office Action dated May 26, 2006 with English translation.  
 Liu, J. et al. "Fullerene Pipes," Science, vol. 280, pp. 1253-1256 (May 22, 1998).  
 Ren, Z.F. et al. "Synthesis of Large Arrays of Well-Aligned Carbon Nanotubes on Glass," Science, vol. 282, pp. 1105-1107 (Nov. 6, 1998).  
 Li, W.Z. et al. "Large-Scale Synthesis of Aligned Carbon Nanotubes," Science, vol. 274, pp. 1701-1703 (Dec. 6, 1998).  
 Tans, Sander J. et al. "Individual single-wall carbon nanotubes as quantum wires," Nature, vol. 386, pp. 474-477 (Apr. 3, 1997).  
 Fan, S. et al. "Self-Oriented Regular Arrays of Carbon Nanotubes and Their Field Emission Properties," Science, vol. 283, pp. 512-514 (Jan. 22, 1999).  
 Bower, C. et al. "Nucleation and growth of carbon nanotubes by microwave plasma chemical vapor deposition," Applied Physics Letters, vol. 77, No. 17, pp. 2767-2769 (Oct. 23, 2000).  
 Merkulov, Vladimir I. et al. "Sharing carbon nanostructures by controlling the synthesis process," Applied Physics Letters, vol. 79, No. 8, pp. 1178-1180 (2001).  
 Teo, KBK et al. "Plasma enhanced chemical vapour deposition carbon nanotubes/nanofibres—how uniform do they grow?," Institute of Physics Publishing, Nanotechnology 14, pp. 204-211 (2003).  
 Tsai, C.L. et al. "Bias effect on the growth of carbon nanotips using microwave plasma chemical vapor deposition," Applied Physics Letters, vol. 81, No. 4, pp. 721-723 (2002).  
 Dean, Kenneth A. et al. "The environmental stability of field emission from single-walled carbon nanotubes," Applied Physics Letters, vol. 75, No. 19, pp. 3017-3019 (1998).  
 Mackie, W.A. et al. "Emission and Processing Requirements for Carbide Films on MO Field Emitters," Mat. Res. Soc Symp. Proc. vol. 509, pp. 173-178 (1998).  
 Rouse, Ambrosio A. et al. "Field emission from molybdenum carbide," Applied Physics Letters, vol. 76, No. 18, pp. 2583-2585 (2000).  
 Adachi, Hiroshi et al. "Stable carbide field emitter," Applied Physics Letters, vol. 43, No. 7, pp. 702-703 (1983).  
 Gilmour, Jr., A.S. Microwave Tubes, Chapter 8, "Gridded Tubes," Artech House, pp. 191-313 (1986).  
 Huang, Michael H. et al. "Room-Temperature Ultraviolet Nanowire Nanolasers," Science, vol. 292, pp. 1897-1899 (2001).  
 Aggarwal, S. et al. "Spontaneous Ordering of Oxide Nanostructures," Science, vol. 287, pp. 2235-2237 (2000).  
 Luo, Yun et al. "Nanoshell tubes of ferroelectric lead zirconate titanate and barium titanate," Applied Physics Letters, vol. 82, No. 10, pp. 1613-1615 (2003).  
 Kong, Y.C. et al. "Ultraviolet-emitting ZnO nanowires synthesized by a physical vapor deposition approach," Applied Physics Letters, vol. 78, No. 4, pp. 407-409 (2001).  
 Aug. 7, 2000 Applied Physics Letters; vol. 77, No. 6; Plasma-induced alignment of carbon nanotubes; pp. 830-832.  
 Jul. 21, 2003 Applied Physics Letters, vol. 83, No. 3; Nanoshell tubes of ferroelectric lead zirconate titanate and barium titanate; pp. 440-442.  
 Jul. 24, 2000 Applied Physics Letters; vol. 85, No. 4; New Mechanism for Electron Emission from Planar Cold Cathodes: The Solid-State Field-Controlled Electron Emitter; pp. 864-867.

\* cited by examiner

FIG. 1(a)



FIG. 1(b)



FIG. 1(c)



FIG. 2(a)



FIG. 2(b)



FIG. 2(c)



FIG. 3(a)



FIG. 3(b)



FIG. 3(c)



FIG. 3(d)



FIG. 4(a)



FIG. 4(b)



FIG. 4(c)



FIG. 4(d)



FIG. 5(a)



FIG. 5(b)



FIG. 6



FIG. 7



FIG. 8



FIG. 9(a)



FIG. 9(b)



## 1

## ARTICLE COMPRISING METAL OXIDE NANOSTRUCTURES

## CROSS REFERENCE TO RELATED APPLICATIONS

This is a Divisional Application of application Ser. No. 11/059,784, filed Feb. 17, 2005, now U.S. Pat. No. 7,276,389 which is an U.S. nonprovisional patent application claiming priority under 35 U.S.C. §119 to U.S. Provisional Application No. 60/547,689, filed on Feb. 25, 2004, the contents of both of which are hereby incorporated by reference in their entirety.

## FIELD OF THE INVENTION

This invention relates to metal oxide nanostructures such as tubes and cones, and, in particular, to such structures made using carbon nanostructures as templates.

## BACKGROUND OF THE INVENTION

Metal oxides have a great potential in various applications due to their interesting physical properties, such as superconducting, semiconducting, ferroelectric, piezoelectric, pyroelectric, ferromagnetic, optical (electro-optic, non-linear optic, and electrochromatic), resistive switching, and catalytic behaviors. Nano-scaled oxide materials have attracted great interest in the last decade because they can exhibit different physical properties than their bulk counterparts. See U.S. Pat. No. 6,036,774 by Lieber, et al. "Method of producing metal oxide nanorods" issued on Mar. 14, 2000; Huang et al., SCIENCE, Vol. 292, p. 1897 (2001); Aggarwal et al., SCIENCE, Vol. 287, p. 2235 (2000); Li et al., Applied Physics Letters, Vol. 82, p. 1613 (2003); Luo et al., Applied Physics Letters, Vol. 83, p. 440 (2003). The oxide nanostructures were prepared by several growth techniques: laser ablation, sputtering, chemical vapor deposition, sol-gel, and molecular-beam-epitaxy. One of the simplest methods is to prepare the nanostructures, such as nanorods, in a tube furnace by the 'vapor-liquid-solid' mechanism suggested by Lieber et al.

Huang et al. demonstrated room-temperature ultraviolet lasing in ZnO nanowire arrays. The nanostructures were used as an optical cavity for lasing. Aggarwal et al. suggested their spontaneously formed oxide "nano-tip" array as a possible candidate for field emission applications. Li et al. presented an approach to use individual  $In_2O_3$  nanowire transistors as chemical sensors, where ultrahigh surface-to-volume ratios were expected to improve the sensitivity. Luo et al. fabricated ferroelectric nanoshell tubes using Si and alumina hole arrays as templates. The nanoshell tubes could be useful for nano-electromechanical system. These results show that nanostructures can be useful for their unique structural advantages.

Carbon nanostructures, such as nanotubes, nanofibers and nanocones, (collectively "CN") and their peculiar characteristics, such as field emission and field effect transistor effects, have also evoked great attention. In recent years, growth techniques for CN were intensively investigated and relatively well established. See Ren et al., SCIENCE, Vol. 282, p. 1105 (1998); Bower et al., Applied Physics Letters, Vol. 77, p. 830 (2000); Merkulov et al., Applied Physics Letters, Vol. 79, p. 1178 (2001); Tsai et al., Applied Physics Letters, Vol. 81, p. 721 (2002); Teo et al., Nanotechnology, Vol. 14, p. 204 (2003).

High-quality single-walled carbon nanotubes are typically grown as randomly oriented, needle-like or spaghetti-like, tangled nanowires by laser ablation or arc techniques (a chemical purification process is usually needed for arc-gen-

## 2

erated carbon nanotubes to remove non-nanotube materials such as graphitic or amorphous phase, catalyst metals, etc.). Chemical vapor deposition (CVD) methods such as used by Ren et al., Bower et al., and Teo et al. tend to produce multi-wall nanotubes attached to a substrate, often with a semi-aligned or aligned, parallel growth perpendicular to the substrate. Also Merkulov et al., Tsai et al., and Teo et al. demonstrated that carbon nanofibers and nano-cones can be grown in optimum conditions, for example by varying gas ratio and voltage bias.

As described in the cited articles, catalytic decomposition of hydrocarbon-containing precursors such as ethylene, methane, or benzene produces CN when the reaction parameters such as temperature, time, precursor concentration, flow rate, are optimized. Catalyst layers such as thin films of Ni, Co, Fe, etc. are often patterned on the substrate to obtain uniformly spaced CN array. Furthermore, the patterning of catalysts makes it possible to tailor the geometry (diameter controlled by catalyst size, height controlled by deposition time) of CN the demands for various applications. The catalyst dots can be patterned by various techniques: self-assembly, unconventional lithography (for example, nano-sphere lithography), and e-beam lithography. Careful patterning and growth enables production of carbon nanotubes with remarkable uniformity in diameter and height (standard deviations ~5%), as reported by Teo et al.

While oxide nanostructures can be fabricated using various available techniques, the most frequently desired structural configurations such as well-defined, vertically aligned and periodically spaced nano oxide wires are not easily obtainable. In addition, some of the unique structures, such as a hollow oxide nanotubes and hollow oxide nanocones, are not easily synthesized using conventional techniques. Accordingly there is a need for improved methods of making oxide nanostructures.

## SUMMARY OF THE INVENTION

This application discloses convenient and novel processing techniques of fabricating oxide nanostructures, some in the form of surface coating, some in the form of nanocomposites, and some in the form of oxide nanotubes or nanocones. The techniques utilize aligned carbon nanotubes or nanocones as growth templates. The carbon template is optionally burned away by heat treatment in an oxidizing atmosphere to create hollow and open oxide nanotubes or nanocones. The resulting novel structures can be useful for articles and devices such as nano sensor arrays, field emission devices such as field emission displays, nanoscale ferromagnetic or ferroelectric memories, nano-reactors, nano catalyst arrays, fuel cells, room temperature UV lasers for higher optical memory density, and nano-electromechanical devices.

## BRIEF DESCRIPTION OF THE DRAWINGS

For a better understanding of the invention, exemplary embodiments are described in connection with the accompanying drawings, in which:

FIGS. 1(a), 1(b) and 1(c) schematically illustrate an exemplary fabrication process for an oxide nanotube array using carbon nanotube/nanofiber array as a template:

FIG. 1(a) illustrates the preparation of a carbon nanotube/nanofiber array,

FIG. 1(b) illustrates the deposition of a metal thin film, and

FIG. 1(c) illustrates an oxidation to form a metal oxide nanotube/nanofiber array;

FIGS. 2(a), 2(b) and 2(c) schematically show a fabrication process for an oxide nano-cone array using carbon nano-cone array as a template:

FIG. 2(a) illustrates the preparation of a carbon nano-cone array;

FIG. 2(b) illustrates the deposition of a metal thin film, and

FIG. 2(c) illustrates an oxidation to form a metal oxide nano-cone array;

FIGS. 3(a) through 3(d) schematically illustrate an exemplary fabrication process for an oxide nanotube array without catalyst particles:

FIG. 3(a) illustrates the preparation of carbon nanotubes/nanofibers,

FIG. 3(b) illustrates selective etching (wet-etching or dry-etching) of a catalyst nano-particle,

FIG. 3(c) illustrates the deposition of a metal thin film, and

FIG. 3(d) illustrates an oxidation to form a metal oxide nanotube and removal of an inside carbon template by burning away;

FIGS. 4(a) through 4(d) schematically show an exemplary fabrication process for an oxide nano-cone array without catalyst particles:

FIG. 4(a) illustrates the preparation of carbon nano-cones

FIG. 4(b) illustrates selective etching (wet-etching or dry-etching) of a catalyst nano-particle,

FIG. 4(c) illustrates the deposition of a metal thin film, and

FIG. 4(d) illustrates an oxidation to form a hollow metal oxide nano-cone;

FIGS. 5(a) and 5(b) illustrate cross-sectional views of a metal oxide nanostructure before and after oxidation, respectively;

FIG. 6 is a cross-sectional view of a nano-tip oxide field emitter;

FIG. 7 illustrates a schematic field emission display using the aligned oxide nanostructure array;

FIG. 8 illustrates an example of a nano sensor array; and

FIGS. 9(a) and 9(b) illustrate UV laser emitters comprising aligned ZnO nanostructures with the carbon template inside the ZnO nanostructures and with the ZnO nanostructures only having the carbon removed, respectively.

It is to be understood that these drawings are for the purposes of illustrating the concepts of the invention and are not to scale.

## DETAILED DESCRIPTION

In the prior art, a variety of quasi-one-dimensional oxide nanostructures, such as nanorods, nanowires and nanobelts, have been fabricated. The synthesis commonly involves a vapor phase (e.g., growth by laser ablation or chemical or physical vapor deposition), and a vapor-liquid-solid (VLS) mechanism. In this growth mode, a liquid metal cluster acts as an energetically favored site for the absorption of gas-phase reactants. The cluster supersaturates and grows into a one-dimensional wire of the material with the alloy cluster atop the wire. The resulting wire morphology depends on experimental parameters such as temperature, pressure, and the nature of the metal catalyst. As suggested by Lieber et al., VLS can be employed to grow various metal oxide materials. Several oxide nanostructures were also prepared by chemical vapor deposition, sol-gel, molecular-beam-epitaxy, and other techniques. However, the use of chemical processes to fabricate oxide nanostructures often introduces many difficult to control processing variables, requires chemically toxic gases, and results in unoriented, randomly distributed nanostructures.

In order to overcome these problems, the present invention employs novel physical vapor deposition processes. To realize useful devices, it is often required to control alignment, geometry, and growth location of nano-features. To achieve such a structure in metal oxide nanostructures, the inventive process utilizes substrate-supported carbon nanostructures (such as nanotubes and carbon nanocones) as templates. The preferred carbon nanostructures are nanostructures such as nanotubes, nanocones and nanowires that project outwardly from the substrate surface. This process uses the fact that carbon nanostructure aligned growth has been well established, often without involving toxic gases. Growth of the carbon nanostructures at specific location can be achieved by patterning of catalyst metal islands. Also, controlling the diameter of the catalyst islands enables one to obtain the nanostructures with desired diameter.

Referring to the drawings, FIG. 1 illustrates an exemplary, versatile and simple fabrication technique for growing an oxide nanotube array 10 by a physical vapor deposition. A carbon nanotube/nanofiber array 10 supported by a substrate 11 can be prepared by conventional CVD technique (FIG. 1(a)). If patterning of catalyst dots is used, a regularly spaced array of nanotubes 12 can be obtained. The patterning also enables one to control the geometry (diameter controlled by catalyst size, height controlled by deposition time) of carbon nanotubes/nanofibers 12. See Teo et al. cited above. Instead of conventional lithography (e-beam lithography and photolithography), some cost-effective patterning methods, such as self-assembly, polymeric approach, nano-sphere lithography, and shadow mask technique also can be used to prepare catalyst island array for growing the nanotube array 10.

The next step of the processes to form the oxide nanostructures is to deposit a thin film 13 of a metal A on the surface of the carbon nanotubes/nanofibers 12 in the array 10 (FIG. 1(b)), for example using sputtering, evaporation or even CVD. Because of the shadow effect by neighboring nanotubes, it is difficult to uniformly coat the nanotubes/nanofibers 12 especially if the length-to-diameter aspect ratio is high. In this case, source beam is 14 desirably obliquely incident on the substrate and rotation of the substrate is also utilized. When the mean free path of molecules is much smaller than the distance between the source and the substrate (like a typical sputtering environment), such a shadowing effect is much smaller than in the case of evaporation processes.

The third step is to oxidize the coated metal layer on the nanotube array. The metal (A) can be oxidized to form metal oxide ( $A_M O_N$ ) by heating the sample in oxygen ambient atmosphere containing, for example, oxygen gas, atomic oxygen, ozone, oxygen plasma,  $NO_2$ , and  $N_2O$ . A partial atmosphere such as incorporating inert gas may also be used. The desired oxidizing temperature is typically in the range of 200-2000° C., preferably in the range of 400-1400° C. The desired heat-treatment time is in the range of 1 second to 500 hours, preferably 10-600 minutes. The completed structure is an oxide-coated carbon nanostructure 15, the surface oxide of which can be utilized for a variety of devices dependent on aligned nanoscale oxide configuration. An alternative way of creating the oxide coating on the CN surface, is to directly deposit oxide material, for example, by using a RF (radio frequency) sputtering or CVD.

An alternative configuration of the inventive oxide nanostructure is to remove all or a part of the carbon nanostructure (CN) template underneath. For some device applications, removal of the carbon simplifies the structure and minimizes a possible complication arising from the presence of carbon, especially since the carbon is electrically conductive while

the oxide is often dielectric. Such a carbon-free oxide nano-structure array can be accomplished by exposing the carbon underneath to an oxidizing atmosphere during heat treatment and burning away the carbon as CO or CO<sub>2</sub> gas.

In order to effectuate such a removal, the metal (or metal oxide) coating is made to be semi-permeable to gases (O<sub>2</sub>, CO or CO<sub>2</sub>). Such a semi-permeable coating can be provided by a careful control of the metal coating process and thickness. A relatively fast deposition or lower temperature deposition of metals tends to create less dense structure. The permeable coating structure has a density of less than 96%, preferably less than 90%.

An alternative process to allow access of oxygen to the carbon is to remove a part of the metal coating (or metal oxide coating) at the upper-end portion of the coated CN structure to expose the carbon. Such an exposed structure is obtained by plasma etching, for example using an oxide plasma. The structure is then subjected to an oxidizing heat treatment. During this oxidation, carbon nanotubes/nanofibers are etched away as carbon oxide gas. Thus a metal oxide (A<sub>M</sub>O<sub>N</sub>) nanotube 15 array can be obtained (FIG. 1(c)). The application is not limited to binary oxides. If the deposited metal is an alloy (e.g., A<sub>L</sub>B<sub>M</sub>), a complex oxide of, A<sub>L</sub>B<sub>M</sub>O<sub>N</sub> can be obtained.

Exemplary oxide nanostructures that can be fabricated according to the inventive processes include semiconducting or dielectric oxides such as ZnO, TiO<sub>2</sub>, MnO<sub>2</sub>, SnO, ZrO<sub>2</sub>, V<sub>2</sub>O<sub>5</sub>, SiO<sub>2</sub>, Cr<sub>2</sub>O<sub>3</sub>, Cr<sub>2</sub>O<sub>3</sub>, MgO, Al<sub>2</sub>O<sub>3</sub>, ferroelectric oxides (such as BaTiO<sub>3</sub>, (Pb,La)(Zr,Ti)O<sub>3</sub>, SrBi<sub>2</sub>Ta<sub>2</sub>O<sub>9</sub>, and (Bi,La)<sub>4</sub>Ti<sub>3</sub>O<sub>12</sub>), magnetic oxides (such as magnetite, Ba-ferrite, Ni-Zn ferrite), superconductive oxides (such as YBa<sub>2</sub>Cu<sub>3</sub>O<sub>7</sub>), and magneto-resistive oxides (such as La-Ca-Mn-O or La-Sr-Mn-O).

FIGS. 2(a)-(c) illustrate an inventive process of fabricating a metal oxide nano-cone array. Most of the processing principles are similar to those for the nanotube array described above. In this case, carbon nano-cone array 20 is used as a permanent or a sacrificial template. The geometry of the cones 21 with the slanting side illustrated in FIG. 2 is especially advantageous, as compared to the nanotube or nanofiber configuration of FIG. 1, in that the deposition of metal 22 becomes much easier and convenient as a standard, vertical deposition can be employed, thus omitting the oblique incident beam arrangement and the substrate rotation. The metal 22 is then oxidized to a metal oxide layer 23 as shown in FIG. 2(c). The carbon nanocone template may be left as a permanent base or the carbon can be burned away using an oxidizing heat treatment similarly as in the case of carbon nanotube or nanofiber removal discussed earlier. Semi-permeable metal coating or plasma etching removal of metal from a small area near the cone tips may be employed.

As the nanocone fabrication steps often involve high temperature CVD processing at several hundred degrees centigrade, it is noted that depending on the specifics of nanotube fabrication, the carbon nanocones sometimes contain a varying amount of other elements such as silicon or oxygen diffused from the silicon or silicon oxide substrate into the nanocone structure during the high temperature fabrication. Allowable types of other elements in the nanocones (and in nanotubes but with a much less extent) include Si, Ga, As, Al, Ti, La, O, C, B, N, and other substrate-related elements. The amount of such elements can be very small or substantial depending on the temperature, time, and electric field applied during the CVD processing, for example in the range of 0.5 to 70 atomic percent.

During the growth of CN, catalyst particles are sometimes retained at the tip. In most cases, the catalyst particles are

transition metals and they are readily oxidized. For some applications, it will be necessary to remove this oxide of transition metal in order to avoid possible device performance complications. To meet such a need, a modified fabrication method is disclosed as shown in FIG. 3. Here carbon nanotubes/nanofibers 30 are prepared (FIG. 3(a)) and an etching step to remove the catalyst nano-particles 31 is applied before deposition of a metal thin film 32 (FIG. 3(b)). Etching of the catalyst metal particle 31 (typically Ni, Fe or Co for carbon nanotube growth) can be done by either dry etching (e.g., fluorine-based reactive ion etching or oxygen plasma etching) or wet etching (e.g., using a solution of phosphoric acid and nitric acid). Once the catalyst metal particles are removed, subsequent processes of metal thin film deposition (FIG. 3(c)) and oxidation (FIG. 3(d)) are carried out to form a final structure of an array of oxide nanotubes. A similar process can be applied to nano-cones 40 as illustrated in FIG. 4.

FIGS. 5(a) and 5(b) schematically illustrate cross-sections of the nanotube tip geometry before and after oxidation, respectively. The diameter of the open end 50 of a nanotube or nanowire 51 can be reduced after oxidation of metal 52 due to the addition of oxygen, and can even be completely closed by the metal oxide 53 if the catalyst particles (not shown) are small and the deposited metal film has a large volume expansion ratio during oxidation. Such a closed or semi-closed tip structure can be useful for special nanostructure array applications, for example, to store liquid, gas, or pharmaceutical drug before the moment of device operation. Fuel storage (such as liquid fuel or hydrogen for fuel cells) or drugs for controlled delivery are some applications.

The oxide nanostructure array has several desirable characteristics particularly useful for device applications. They include the very large surface area associated with the nanoscale and vertically elongated structure, which can be useful for enhancing the kinetics chemical, catalytic or other reactions. The sharp tip configuration with high aspect ratio, in combination with a vertically aligned and laterally spaced array structure can be useful for electron field emitter applications. The cone-shaped configuration provides mechanical sturdiness of the nanostructure, much better than in the case of the nanotube or nanofiber configuration. The hollow inside in some of the inventive configurations (when the carbon template is burned away) can provide many, nanoscale storage reservoirs for liquid or gaseous fuel, medicine, chemical reactant, and catalysts for nanoscale chemical reactors or sensor applications. The presence of many nanoscale and periodically placed nanoscale oxide elements can also be utilized for ferroelectric or ferromagnetic memory applications. Some of these device applications are described below.

#### 50 Nano-Tip Field Emitters

In vacuum microelectronics, great attention has been paid on the application of field-emitters to flat-panel field-emission displays (FED's), RF amplifiers, multi-beam electron-beam lithography, specialty lamps, and nanoscopic X-ray sources. All of these require stable field emitters with sufficiently large emission current.

An important issue in field emitters is their stability with the residual ambient gas. Particularly important is that the field emitter tips made of refractory metals like molybdenum, niobium, and tungsten are susceptible to oxidation. Such field emitters were disclosed by Chalamala et al. in U.S. Pat. No. 6,091,190, "Field emission device", issued on Jul. 18, 2000. In the present invention, sharp metal (e.g., Mo) tip field emitters can have a novel surface passivation layer made from 60 oxides of one of the metals selected from Ba, Ca, Sr, In, Sc, Ti, Ir, Co, Sr, Y, Zr, Ru, Pd, Sn, Lu, Hf, Re, La, Ce, Pr, Nd, Pm, Sm, Eu, Gd, Tb, Dy, Ho, Er, Tm, Yb, Th, and combinations

thereof. The oxide is helpful in improving the emission stability. Moreover its work function is less than that of molybdenum.

Referring to the drawings, FIG. 6 is a schematic cross-sectional illustration of an exemplary inventive field emitter, which is prepared by using a carbon nanocone **61** (which can be removed if desired) as a template. The field emitter **60** comprises two layers, an oxide passivation layer ( $A_MO_N$ ) **62** and metal layer **63** (e.g., Mo). This structure can be fabricated following the process shown in FIG. 2, but multilayer of A/Mo should be grown on the carbon nano-cones in the step corresponding to FIG. 2(b). An ensuing oxidation step can oxidize top-most metal (A) layer to form oxide ( $A_MO_N$ ). Carbon nanotubes/nanofibers also can be used as templates and similar process can be applied to prepare tube-type nano-tip array, as illustrated in FIG. 1.

The inventive ‘nano-tip field emitters’ is a robust electron source, since it takes the advantages from both the carbon nano-cone (high aspect ratio and sharp tip geometry useful for electric field concentration) and the passivated Spindt-type emitter (high tolerance in ambient). Such a high aspect ratio can greatly reduce the turn-on voltage for field emission. Metal (e.g., Mo) films or underlying carbon can provide a good conduction path for electron transport during electron emission, which can produce a large emission current.

A field emission display device incorporating the inventive field emitter array is schematically illustrated in FIG. 7. The display device of FIG. 7 uses one or more arrays **70** of field emitters such is shown in FIG. 6 disposed on a cathode substrate **71** to emit electrons. Emission is partially controlled by respective gate electrode **72** which can be supported overlying the emitters by an insulating pillar **73**. Emited electrons are attracted into collision with an anode/phosphor assembly **74** and the resulting light can be seen through a glass plate **75**.

#### Nano Sensor Array

A sensor array system is useful for clinical, environmental, health and safety, remote sensing, military, food/beverage and chemical processing applications. This array contains several gas sensors, such as metal oxides ( $SnO_2$ ,  $ZnO$ ,  $CdO$ ,  $PbCrO_4$ ,  $Fe_2O_3$ ,  $TiO_2$ ,  $ThO_2$ ,  $MoO_3$ ,  $V_2O_5$ ,  $MnO_2$ ,  $WO_3$ ,  $NiO$ ,  $CoO$ ,  $Cr_2O_3$ ,  $Ag_2O$ ,  $In_2O_3$ , and so on). The sensor array displays the capacity to identify and discriminate between a variety of vapors by virtue of small site-to-site differences in response characteristics. Such a sensor array was disclosed by Hoffheins et al. in U.S. Pat. No. 5,654,497, “Motor vehicle fuel analyzer”, issued on Jun. 3, 1996. Various fabrication methods have been developed, for example, McDevitt et al. in U.S. Pat. No. 6,649,403, “Method of preparing a sensor array” issued on Nov. 18, 2003.

FIG. 8 schematically illustrates an exemplary inventive sensor array **80**, which is prepared by using carbon nanocones as templates. In order to prepare a multifunctional sensor capable of detecting different gas or different physical or chemical stimuli, various kind of metals (A, B, C, . . .) are deposited on different sets of nanocone templates (**81**, **82**, and **83**, respectively) on a wafer. Such a selective deposition can be carried out, for example, by using a shadow mask which allow a selective thin film deposition of metal A (or the oxide  $AO_x$ ) in a rectangular area at the bottom of FIG. 8. The shadow mask is then moved to the middle area rectangle for deposition of metal B (or the oxide  $BO_x$ ). Such a step is repeated in order to produce as many areas as desired for sensing of each specific gas. A metal oxide array obtained by such a processing is illustrated in FIG. 8, which shows an example of nano-cone templates **84** coated with different metal-oxide sensors. A set of electrodes **85** is prepared for each set of metal oxide sensors as shown in FIG. 8. These

electrodes are connected to a detection system for interrogation/analysis of the obtained signals. The large total surface area from many sensor nanowires within each set adds to the total cumulative signal amplitude.

The inventive ‘nano sensor array’ is very sensitive, since it has a ultrahigh surface-to-volume ratio. Moreover, with a nanoscale patterning, a very large number of sensor sets can be incorporated for detection of many different types of chemical or physical stimuli.

The application of the inventive oxide nanostructure array is not limited to a chemical sensor. Resistances of some metal oxides are varied under light (e.g.,  $In_2O_3$ ) or magnetic field (e.g., perovskite manganese oxides such as  $La_{1-x}Ca_xMnO_3$ ). Those materials can be used for photodetectors and magnetic field sensors. Also some metal oxides generate electric current when heat (pyroelectric materials) or pressure (piezoelectric materials) is applied. These properties can be utilized for infrared sensors and pressure sensors. In all these cases, sensitivity of the oxide nanostructure disclosed in this invention is much higher than that for the conventional planar thin films due to its enormous surface area.

The inventive oxide nanostructures can also be useful for optoelectronic applications. For example, it is demonstrated that  $ZnO$  nanowires can produce room temperature UV (ultraviolet) laser. See articles by Y. C. Kong et al, Applied Physics Letters Vol. 78, p. 407 (2001) and M. Huang et al., Science, Vol. 292, p. 1897 (2001).  $ZnO$  is a direct wide-bandgap semiconductor with its bandgap of 3.37 eV at room temperature which is suitable for short wavelength laser or diode applications such as UV or blue emitters. Such short wavelengths can allow higher optical memory densities for CD (compact disk) devices or magneto-optical memory devices. Due to the much larger exciton binding energy of about 60 meV in  $ZnO$  as compared to other large bandgap semiconductors (~25 meV for GaN and ~22 meV for  $ZnSe$ ), the excitons in  $ZnO$  are thermally stable at room temperature thus providing an extra advantage. As illustrated schematically in FIG. 9, an aligned oxide nanostructure **90** comprising the  $ZnO$  coating on the carbon nanotube template **91**, FIG. 9(a), or a similar structure **92** comprising  $ZnO$  nanotubes only after the removal of carbon template inside, FIG. 9(b), can thus be useful as an efficient UV or blue light emitter device.

The aligned oxide nanostructure can also be useful for ferroelectric or ferromagnetic memory devices. An exemplary oxide ferroelectric memory material is barium titanate ( $BaTiO_3$ ), and an exemplary ferromagnetic oxide memory material is barium hexaferrite (Please Check This.  $BaO_6Fe_2O_3$ ). For such memory devices, the gap between the nanowires in the aligned oxide nanostructure of FIG. 1(b) or FIG. 1(c) can be filled with nonfunctional materials such as a polymer or physically deposited (e.g., by RF sputtering) aluminum oxide, then the top surface is polished flat (e.g., by chemical mechanical polishing technique), and electrodes as well as electrical or magnetic interrogation circuits are added so as to induce or detect changes in stored electrical charge or magnetic moment.

The inventive nano oxide arrays such as solid, composite or hollow nanowire or nanocone array of oxides are also useful for other device applications such as nano-reactors, nano catalyst arrays, fuel cells, and nano-electromechanical devices.

It can now be seen that one aspect of the invention is a method of making an array of metal oxide nanostructures comprising the steps of providing a substrate including an array of projecting carbon nanostructures and forming a metal oxide coating overlying the surface of the carbon nanostructures. The metal oxide coating can be formed by depos-

iting the metal and oxidizing the deposited metal to form the array of metal oxide nanostructures. Or the metal oxide coating can be deposited overlying the carbon nanostructures. The substrate typically has a major surface and the carbon nanostructures are advantageously disposed in a two dimensional array on the surface. Preferably the carbon nanostructures are disposed in a substantially equal spaced, spaced-apart array as by appropriate disposition of catalyst islands, and they may advantageously have substantially uniform height above the substrate. The remains of the catalyst islands can be etched away after carbon nanostructures are grown. The projecting carbon nanostructures can be nanotubes, nanowires or nanocones.

In depositing the metal coating or the metal oxide coating, the material may be deposited at an oblique angle to the substrate surface, and the substrate surface can be rotated to reduce shadowing of nanostructures by neighboring nanostructures.

Deposited metal can be oxidized by heating in an oxidizing gas ambient at a temperature in the range 200-200° C. for 1 second to 500 hrs. and preferably at a temperature in the range 400-1400° C. for 10 to 600 minutes. The metal can be an elemental metal or an alloy. Typical useful metals include Zn, Ti, Mn, Sn, Zr, V, Si, Cr, Mg, Al, Fe, Ba, Fb, La, Sr, Bi, Ta, Cu, Ca and their alloys.

After the carbon nanostructures have served as a template for the formation of metal or metal oxide coatings, the carbon can be removed as by heating in an oxidizing atmosphere.

Another aspect of the invention is the resulting article comprising a substrate including an array of projecting metal oxide nanostructures. The oxide nanostructures can be in the form of nanotubes, nanocones or nanowires. The nanostructures can be disposed in a spaced-apart two dimensional array, preferably with substantially equal spacing and substantially uniform height above the substrate. The article can be, among other things, a field emission structure using the oxide nanostructures as nanotip field emitters. It can also be used as a nanosensor array.

It is understood that the above-described embodiments are illustrative of only a few of the many possible specific embodiments which can represent applications of the invention. Numerous and varied other arrangements can be made by those skilled in the art without departing from the spirit and scope of the invention.

What is claimed is:

1. A field emission device comprising:

a plurality of field emitters on a cathode substrate to emit electrons, the plurality of field emitters including a plurality of nanocones having an abscised tip;

a gate electrode overlying the plurality of field emitters to partially control emission from the plurality of field emitters; and

an anode/phosphor assembly positioned for receiving emitted electrons,

wherein the plurality of nanocones are supported by and projecting from at least two regions of the cathode substrate and include an oxidized metal shell having an empty core on the entire surfaces of each nanocone, the oxidized metal shell including a refractory metal between a first metal oxide and a second metal oxide, the refractory metal including molybdenum, niobium, and tungsten.

2. The field emission device of claim 1, wherein the plurality of field emitters each include a metal film between the oxidized metal shell coated on the entire surfaces of the plurality of nanocones.

3. The field emission device of claim 1, further comprising: two insulating pillars on the cathode; and a glass plate on the anode/phosphor assembly, wherein an array of the plurality of field emitters are between the two insulating pillars,

the gate electrode includes two gate electrodes that are on the two insulating pillars respectively, and the anode/phosphor assembly is over at least one of the cathode, the two gate electrodes, and the array of the plurality of field emitters.

4. The field emission device of claim 3, wherein a plurality of arrays of the plurality of field emitters are on the cathode.

5. The field emission device of claim 1, wherein the oxidized metal shell coated on the plurality of nanocones includes an oxide of one of Ba, Ca, Sr, In, Sc, Ti, Ir, Co, Sr, Y, Zr, Ru, Pd, Sn, Lu, Hf, Re, La, Ce, Pr, Nd, Pm, Sm, Eu, Gd, Th, Dy, Ho, Er, Tm, Yb, Th, and combinations thereof.

6. A sensor array of nanostructures including one or more arrays comprising:

a plurality of nanocones supported by and projecting from at least two regions of a substrate and including an oxidized metal shell having an empty core on the entire surfaces of each nanocone, the oxidized metal shell including a refractory metal between a first metal oxide and a second metal oxide, the refractory metal including molybdenum, niobium, and tungsten, wherein the plurality of nanocones have an abscised tip.

7. The sensor array of claim 6, wherein:

the first metal oxide contains one of a  $\text{SnO}_2$ ,  $\text{ZnO}$ ,  $\text{CdO}$ ,  $\text{PbCrO}_4$ ,  $\text{Fe}_2\text{O}_3$ ,  $\text{TiO}_2$ ,  $\text{ThO}_2$ ,  $\text{MoO}_3$ ,  $\text{V}_2\text{O}_5$ ,  $\text{MnO}_2$ ,  $\text{WO}_3$ ,  $\text{NiO}$ ,  $\text{CoO}$ ,  $\text{Cr}_2\text{O}_3$ ,  $\text{Ag}_2\text{O}$ , perovskite manganese oxides,  $\text{In}_2\text{O}_3$ ; and

the second metal oxide contains a different one of a  $\text{SnO}_2$ ,  $\text{ZnO}$ ,  $\text{CdO}$ ,  $\text{PbCrO}_4$ ,  $\text{Fe}_2\text{O}_3$ ,  $\text{TiO}_2$ ,  $\text{ThO}_2$ ,  $\text{MoO}_3$ ,  $\text{V}_2\text{O}_5$ ,  $\text{MnO}_2$ ,  $\text{WO}_3$ ,  $\text{NiO}$ ,  $\text{CoO}$ ,  $\text{Cr}_2\text{O}_3$ ,  $\text{Ag}_2\text{O}$ , perovskite manganese oxide, and  $\text{In}_2\text{O}_3$ .

8. The sensor array of claim 6, further comprising: a first pair of electrodes electrically connected to the plurality of nanocones on the at least one region of the at least two regions of the substrate; and a second pair of electrodes electrically connected to the plurality of nanocones on the at least one other region of the at least two regions of the substrate.

9. An array of nanostructures comprising:

a plurality of nanocones supported by and projecting from at least two regions of a substrate and including an oxidized metal shell having an empty core on the entire surfaces of each nanocone, the oxidized metal shell including a refractory metal between a first metal oxide and a second metal oxide, the refractory metal including molybdenum, niobium, and tungsten, wherein the plurality of nanocones have an abscised tip.

10. The array of nanostructures according to claim 9, wherein the substrate has a major surface and the plurality of nanocones are disposed in a two dimensional array on the major surface.

11. The array of nanostructures according to claim 9, wherein the oxidized metal shell having an empty core is formed by sputtering, evaporating or chemical vapor disposition.

12. An article comprising:

an array of nanocones supported by and projecting from at least two regions of a substrate and including an oxidized metal shell having an empty core on the entire surfaces of each nanocone, wherein each nanocone includes an oxidized metal shell having an empty core, the oxidized metal shell including a refractory metal

**11**

**12**

between a first metal oxide and a second metal oxide, the refractory metal including molybdenum, niobium, and tungsten, and wherein the array of nanocones have an abscised tip.

**13.** The article of claim **12**, wherein the oxidized metal shell having an empty core includes an oxidized alloy. 5

**14.** The article of claim **12**, wherein distal ends of the array of nanocones are closed.

\* \* \* \* \*